

## UNITED STATES PATENT OFFICE

2,513,391

## WATERPROOF FUSE

Henryk Zenftman, Saltcoats, Scotland, assignor  
to Imperial Chemical Industries Limited, a cor-  
poration of Great Britain

No. Drawing. Application October 6, 1944, Se-  
rial No. 557,559. In Great Britain October 6,  
1943

8 Claims. (Cl. 52--2)

1

The present invention relates to the manufacture of non-detonating fuses for blasting and the like operations, and more especially of safety fuse, of the kind in which the core of self-combustible material enclosed in the envelope comprises a coherent rod of imporous composition formed by an extrusion of the composition in a thermoplastic condition.

Although safety fuse is usually made by enveloping a stream of a loose blackpowder composition in a suitable textile envelope, passing the resulting core through a die and applying waterproof coatings, fuses having a coherent waterproof core made by extrusion of a thermoplastic mixture containing nitrocellulose gelatinised with nitroglycerine and suitable pulverulent oxidising and reducing agents have at various times been suggested in order to prevent water leaking through faults in the envelope extinguishing the fuse, but such fuses have hitherto found only limited application on account of their undesirable sensitiveness to friction and shock.

It has also been proposed, in British Patent No. 544,252 (corresponding to U. S. Patent No. 2,363,569, Caldwell, et al.) with similar objects to form a waterproof non-detonating safety fuse of the kind having a coherent imperforate extruded core of plastic material surrounded by an envelope of less combustible or uninflammable material, whereof the core comprises a deflagrating mixture of normally pulverulent oxidising and reducing agents and a non-detonating binding agent therefor, including gelatinised nitrocellulose but free from nitroglycerine, the weight of the binding agent in the core composition being not more than that of the mixture of oxidising and reducing agents.

Unless a volatile solvent for the nitrocellulose is employed, in which case the extruded core must be exposed for a long period in order to evaporate off the solvent, before the outer coverings are applied, the incorporation of the mixture of pulverulent oxidising and reducing agents with the binding agent containing the nitrocellulose gelatinised with a plasticiser, and also the extrusion of the resulting composition, must be carried out at a high temperature in order to render the composition workable. Nitrocellulose is itself a self-combustible material having an unusually low spontaneous ignition temperature, and the spontaneous ignition temperature of the core composition is substantially lower than that of any mixture of pulverulent oxidising and reducing agents that would in practice be used in it. These manufacturing operations are

therefore attended by a substantial fire risk, and the gelatinisation of the nitrocellulose with the plasticiser is also attended by a certain hazard. Moreover, in the case of certain inorganic oxidising agents the difficulty is frequently encountered that they cause the binding power of the nitrocellulose plastic to deteriorate more or less rapidly at the high temperatures used:

We have now found that serviceable or improved fuses of the kind described can be produced with greater safety or with greater facility from pulverulent oxidising and reducing agents capable of reacting with sufficient vigour, if the thermoplastic binding agent with which they are made into a plastic at raised temperature is a composition that is based upon a water insoluble resinous polymerised unsaturated compound, and becomes fluent at a temperature between about 90° and about 125° C.

According to the present invention a non-detonating fuse of the kind described comprises a thermoplastic binding agent comprising a water-insoluble resinous polymerised unsaturated compound which becomes fluent at a temperature between about 90° and about 125° C. and a mixture of pulverulent oxidising and reducing agents capable of reacting therein with such intensity as to permit continuous propagation of combustion.

The water-insoluble resinous polymerised unsaturated compound may be, for instance, a polymerised ester or nitrile of acrylic or methacrylic acid, a polymerised vinyl ester of an inorganic acid, a polyvinyl acetal, or a polymerised unsaturated hydrocarbon such as polystyrene or polymerised ethylene. A plasticiser for the polymerised unsaturated compound may be included in the composition. Normal phthalic esters or phosphoric esters may be used.

A suitable mixture of pulverulent oxidising and reducing agents is one comprising silicon and a lead compound thermally decomposable to yield products comprising lead monoxide and free oxygen. Examples of such lead compounds are the higher oxides of lead as, for example red lead and lead peroxide, and lead nitrate. Substantially gasless mixtures can, for instance be obtained from red lead and silicon, which desirably contain an excess of silicon up to about 25% on the stoichiometric mixture. If desired, these mixtures may be modified by the substitution of potassium nitrate or barium nitrate for a portion of the lead compound as the oxidising constituent of the mixture, wherein for example there may be conveniently present not less than about

1.5 parts red lead per part of potassium nitrate, and an excess of silicon on the stoichiometric mixture. These modified compositions are not of course gasless, but somewhat slower burning fuses can be obtained from them than from the mixtures based on red lead and silicon alone.

In putting the invention into effect, the pulverulent oxidising and reducing agents are worked with the thermoplastic binding agent to form the core composition at a temperature between about 90° and 125° C., the temperature being sufficient to confer the necessary fluency on the binding agent, and the core composition so obtained is extruded at a suitably elevated temperature, the temperature being not higher than about 125° C. Temperatures of a range from about 100-120° C. are usually convenient to employ in carrying out these operations, the temperature of extrusion being the higher of the two.

In general the speed of a fuse prepared from a given mixture of oxidising and reducing agents according to the present invention is slower than that of a fuse prepared from the same mixture of oxidising and reducing agents with a plasticised nitrocellulose binder; and the higher the proportion of binding agent to the mixture, the lower the speed of the fuse. An important safety advantage is that the flame does not race from end to end of the core made according to the invention even if the envelope is not closely applied. The speed of the fuse may be somewhat increased by extruding the core composition around a soft metal wire, for instance, a copper wire of 20-40 Standard wire gauge diameter.

In making up the core composition, it is usually preferable to work either the pulverulent oxidising agent or the pulverulent reducing agent into the thermoplastic binding agent, and subsequently work in the pulverulent reducing agent or oxidising agent component as the case may be, rather than work in a pulverulent mixture of the oxidising and reducing components, or rather than work both pulverulent components in simultaneously.

Thermoplastic binding agents based on resinous polymerised unsaturated compounds frequently have better binding properties than those based on nitrocellulose, so that a higher proportion of the pulverulent ingredients can be used in making up the core composition according to the present invention. The density of the pulverulent ingredients has a considerable influence on the amount of the thermoplastic binding agent required, the denser the composition the less binding agent being required. For instance in the case of the aforesaid mixtures of pulverulent oxidising and reducing agents comprising red lead as an oxidising ingredient, a thermoplastic binding agent composed of approximately equal parts of polymethyl methacrylate and dibutyl phthalate is capable of binding from about 6.7 to 8.3 times its weight of the pulverulent mixture, whereas a thermoplastic binding agent composed of equal parts of industrial nitrocellulose and dibutyl phthalate can only bind about half of these amounts, the oxidising and reducing agents being in each case mixed into the thermoplastic binding agent in a low pressure steam heated mixer and yielding a core composition that can be satisfactorily extruded from a machine having an extrusion head heated to the same temperature. In these mixtures the red lead is the most dense of the pulverulent ingredients.

In fuses of the kind described made with a thermoplastic binding agent comprising a plasticised nitrocellulose composition, the binding agent takes a prominent part in the combustion of the core and is substantially burned away to form gaseous products, but in the fuses made according to the present invention the evidence provided by the products of the destructive distillation of the core composition as the fuse burns indicates that the binding agent undergoes little actual combustion.

The fact that according to the present invention a higher proportion of pulverulent oxidising and reducing agents can be included in the composition of the core and the fact that the binding agent is less effectively consumed as the fuse burns, than in the case of fuse of the kind described made with a thermoplastic binding agent based on nitrocellulose, facilitate the production of fuses yielding a larger amount of ash and a smaller amount of gas from the core. Such fuses are subject to a smaller variation in burning speed under varying atmospheric pressures, and when oxidising and reducing agents that react with a negligible evolution of gas are employed according to our invention, the fuses show very little variation indeed in burning speed with varying pressure. Furthermore, they burn more satisfactorily than prior fuses when immersed in a bulk of water.

It is a further advantage of the invention that the binding power of the resinous polymerised unsaturated compounds is substantially unaffected by the maintenance of the core composition at the elevated temperature at which it is extruded.

The invention is illustrated in the following examples, in which the parts are parts by weight:

#### Example 1

20 parts of silicon sieved to pass through a 200 mesh British Standard specification screen are gradually worked into 12 parts of a thermoplastic binding agent composed of methyl methacrylate polymer 48 per cent and dibutyl phthalate 52 per cent contained in a steam jacketed Werner-Pfleiderer mixing machine, at a temperature of about 100° C., until the silicon is well distributed through the plastic. 80 parts of the red lead powder as used in paints are worked into the plastic, the temperature being allowed to rise to about 110° C. The action of the machine is continued until the red lead is well distributed and the mixture has a coherent plastic consistency.

The resulting composition is transferred to an extrusion machine having a cylindrical die of 0.06 inch diameter heated to about 120° C. When the core so extruded has cooled sufficiently to solidify, a cotton yarn covering and counter- ing are spun round it, and it is coated with bitumen and guttapercha and again countered with cotton yarns and finally coated with a colour varnish made from glue, starch and china clay. The burning speed of the resulting waterproof safety fuse is about 160 seconds per yard at ordinary atmospheric pressure.

#### Example 2

The procedure is the same as in Example 1 except that the ingredients of the core composition are used in the proportions silicon 25 parts, red lead 75 parts and binding agent 13.3 parts.

The burning speed at atmospheric pressure is

about 166 seconds per yard, and at 150 mm. pressure about 176 seconds per yard.

*Example 3*

The quantities and procedure are as in Example 2, except that a 36 Standard wire gauge copper wire is pulled centrally through the die at the same rate that the plastic composition is extruded around it. The burning speed of the resulting safety fuse at atmospheric pressure is about 119 seconds per yard.

*Example 4*

The quantities and procedure are as in Example 1, except that a 36 Standard wire gauge copper wire is pulled centrally through the die at the same rate that the plastic composition is extruded around it. The burning speed of the resulting safety fuse at atmospheric pressure is about 125 seconds per yard.

*Example 5*

The inorganic ingredients are silicon, red lead, and potassium nitrate, of which there are used respectively 23.8 parts, 54.4 parts and 21.8 parts. The red lead and the potassium nitrate, which is screened to pass a 100 mesh British Standard specification screen are mixed together and the mixture is introduced into a hot plastic composition containing 23.8 parts silicon distributed through 13.64 parts of a binding agent composed of methyl methacrylate polymer 48 per cent and dibutyl phthalate 52 per cent. In other respects the preparation of the waterproof safety fuse is carried out as described in Example 1. The burning speed of the resulting fuse at atmospheric pressure is about 190 seconds per yard.

*Example 6*

The ingredients of the core composition are the same as in Example 5, and are present in the proportions, silicon 35.25 parts, red lead 46.25 parts, potassium nitrate 18.5 parts, and binding agent 15.0 parts. The procedure is otherwise the same as in Example 5. The resulting waterproof safety fuse has a burning speed of about 144 seconds per yard at atmospheric pressure.

*Example 7*

The proportions of the ingredients present in the core composition are, silicon 33.6 parts, red lead 52.2 parts, potassium nitrate 14.2 parts, and binding agent 13.0 parts. The procedure is otherwise the same as in Example 5. The burning speed of the resulting waterproof safety fuse at atmospheric pressure is about 121 seconds per yard.

*Example 8*

The proportions of the ingredients present in the core composition are silicon 30.0 parts, red lead 50.0 parts, potassium nitrate 20.0 parts, and binding agent 14.3 parts. A 36 Standard wire gauge copper wire is pulled centrally through the extrusion die at the same rate as the core composition is extruded around it. Otherwise the procedure is the same as in Example 5. The burning speed of the resulting waterproof safety fuse at atmospheric pressure is about 100 seconds per yard.

*Example 9*

The proportions of the ingredients present in the core composition are silicon 25.0 parts, red lead 75.0 parts, and binding agent 13.0 parts.

The core composition is prepared in the manner described in Example 1 and extruded around a 36 Standard wire gauge copper wire, as described in Example 3. A jute covering and a cotton counteracting are then spun around the core when it has cooled sufficiently to solidify, and subsequently the textile covered core is coated by extruding around it a layer of plastic waterproofing composition comprising polyvinyl chloride, dibutyl phthalate and tricresyl phosphate through a suitably heated die. The resulting waterproof safety fuse has a burning speed of about 105 seconds per yard at atmospheric pressure.

*Example 10*

The quantities and procedure are the same in Example 6 except that a 34 instead of a 36 Standard wire gauge copper wire is used. The burning speed at atmospheric pressure is about 90 seconds per yard.

*Example 11*

The proportions of the pulverulent ingredient and the amount are the same as in Example 8, except the type of thermoplastic used as a binding agent which is comprised of 70% of vinyl acetate polymer and 30% dibutyl phthalate. A 33 Standard wire gauge copper wire is pulled centrally through the extrusion die at the same rate as the core composition is extruded around it. Otherwise the procedure is the same as in Example 8.

The burning speed of the resulting safety fuse at atmospheric pressure is about 150 seconds per yard.

*Example 12*

The proportions of the pulverulent ingredient and amounts of binding agents are the same as in Example 8 except that the thermoplastic used as a binding agent, is composed of 65% of vinyl acetate polymer and 30% dibutyl phthalate. A 33 Standard wire gauge copper wire is pulled centrally through the extrusion die at the same rate as the core composition is extruded around it. Otherwise the procedure is the same as in Example 8.

The burning speed of the resulting safety fuse at atmospheric pressure is about 140 seconds per yard.

*Example 13*

The inorganic ingredients are red lead, barium nitrate, and silicon, of which there are used respectively 50 parts, 50 parts and 35 parts. 120 parts of this mixture of inorganic ingredients are homogeneously admixed with 15 parts of a binding agent composed of methyl methacrylate polymer 55% and dibutyl phthalate 45%. In other respects the preparation of the waterproof safety fuse is carried out as described in Example 1. The burning speed of the resulting fuse at atmospheric pressure is 500 seconds per yard.

*Example 14*

The inorganic ingredients are lead nitrate and silicon of which there are used respectively 65 parts, and 35 parts. 90 parts of this mixture of inorganic ingredients are homogeneously admixed with 15 parts of a binding agent composed of polystyrene 65% and dibutyl phthalate 45%. In other respects the preparation of the waterproof safety fuse is carried out as described in Example 1. The burning speed of the resulting fuse at atmospheric pressure is 280 seconds per yard.

I claim:

1. A waterproof non-detonating fuse suitable for blasting and like operations, having a self-combustible core enclosed in a protective envelope, said core being an imporous, coherent, rod-like body of a homogeneous thermoplastic composition comprising a water-insoluble resinous polymerized unsaturated compound which becomes fluent at a temperature between 90° and 125° C. and is not readily combustible, in and throughout which are incorporated and uniformly distributed, in intimate association, normally pulverulent oxidizing and reducing agents comprising a lead compound and silicon, the latter in stoichiometric excess, wherein the oxidizing and reducing agent composition has a relatively low ignition temperature in order to permit continuous propagation of core combustion and said lead compound is thermally decomposable to yield products comprising lead monoxide and free oxygen.

2. A waterproof non-detonating fuse suitable for blasting and like operations, having a self-combustible core enclosed in a protective envelope, said core being an imporous, coherent, rod-like body of a homogeneous thermoplastic composition comprising a water-insoluble resinous polymerized unsaturated compound which becomes fluent at a temperature between 90° and 125° C. and is not readily combustible, in and throughout which are incorporated and uniformly distributed, in intimate association, normally pulverulent oxidizing and reducing agents comprising a lead compound and silicon, the latter in stoichiometric excess, the ignition temperature of the oxidizing and reducing agent composition being relatively low in order to permit continuous propagation of core combustion, and the said lead compound comprising a higher oxide of lead.

lead compound comprising a higher oxide of lead. 3. A waterproof non-detonating fuse suitable for blasting and like operations, having a self-combustible core enclosed in a protective enveloped, said core being an imporous coherent, rod-like body of a homogeneous thermoplastic composition comprising a water-insoluble resinous polymerized unsaturated compound which becomes fluent at a temperature between 90° and 125° C. and is not readily combustible, in and throughout which are incorporated and uniformly distributed, in intimate association, normally pulverulent oxidizing and reducing agents comprising red lead and silicon, the latter in stoichiometric excess, the ignition temperature of the oxidizing and reducing agent composition being relatively low in order to permit continuous propagation of core combustion.

4. A waterproof non-detonating fuse as claimed in claim 3, wherein the water-insoluble resinous polymerized unsaturated compound comprises a plasticized polymerized methyl methacrylate.

5. A waterproof non-detonating fuse suitable for blasting and like operations, having a self-combustible core enclosed in a protective envelope, said core being an imporous, coherent, rod-like body of a homogeneous thermoplastic composition comprising a water-insoluble resinous polymerized unsaturated compound which becomes fluent at a temperature between 90° and 125° C. and is not readily combustible, in and throughout which are incorporated and uniformly distributed, in intimate association, normally pulverulent oxidizing and reducing agents comprising lead nitrate and silicon, the latter in stoichiometric excess, the ignition temperature of the oxidizing and reducing agent composition being relatively low in order to permit continuous propagation of core combustion.

6. A waterproof non-detonating fuse as claimed in claim 1, wherein potassium nitrate is included as a further oxidizing constituent of the mixture.

7. A waterproof non-detonating fuse suitable for blasting and like operations, having a self-combustible core enclosed in a protective envelope, said core being an imporous, coherent, rod-like body of a homogeneous thermoplastic composition comprising a water-insoluble resinous polymerized unsaturated compound which becomes fluent at a temperature between 90° and 125° C. and is not readily combustible, in and throughout which are incorporated and uniformly distributed, in intimate association, normally pulverulent oxidizing and reducing agents comprising a lead compound and silicon, the latter in stoichiometric excess, the ignition temperature of the oxidizing and reducing agent composition being relatively low in order to permit continuous propagation of core combustion, wherein said oxidizing agent comprises red lead and potassium nitrate, there being present not less than about 1.5 parts red lead per part potassium nitrate.

8. A waterproof non-detonating fuse as claimed in claim 1, wherein barium nitrate is included as a further oxidizing constituent of the mixture.

HENRYK ZENFTMAN.

## REFERENCES CITED

The following references are of record in the file of this patent:

UNITED STATES PATENTS

| Number    | Name      | Date           |
|-----------|-----------|----------------|
| 1,805,214 | Hale      | May 12, 1931   |
| 1,877,127 | Hale      | Sept. 13, 1932 |
| 2,165,263 | Holm      | July 11, 1939  |
| 2,349,048 | Mackey    | May 16, 1944   |
| 2,363,569 | Caldwell  | Nov. 28, 1944  |
| 2,407,131 | Bruson    | Sept. 3, 1946  |
| 2,410,801 | Audrieth  | Nov. 12, 1946  |
| 2,416,639 | Pearshall | Feb. 25, 1947  |
| 2,423,427 | Pavny     | July 1, 1947   |